

1

3,657,130  
LIQUID DEVELOPER FOR ELECTRO-  
PHOTOGRAPHY

Hazime Machida, Akira Tsurugi, Zenjiro Okuno, and  
Akinori Mizuno, Tokyo, Japan, assignors to Kabushiki  
Kaisha Ricoh, Tokyo, Japan  
No Drawing. Filed Feb. 3, 1970, Ser. No. 8,398  
Claims priority, application Japan, Feb. 8, 1969,  
44/9,536  
Int. Cl. G03g 9/04  
U.S. Cl. 252—62.1

3 Claims

### ABSTRACT OF THE DISCLOSURE

A liquid developer for electrophotography comprising a carrier liquid and a toner dispersed in said carrier liquid, said toner consisting substantially of finely-divided particles having a definite color, at least one coating agent as coated on the surfaces of said particles and selected from the group consisting of a synthetic rubber, a natural rubber, polycondensates of said two rubbers and vinyl polymers having an insolubility against said carrier liquid, and a graft-polymer having an affinity with said carrier liquid and consisting of at least one vinyl monomer selected from the group consisting of polymeric vinyl monomers, said graft-polymer being graft-copolymerized to said coating agent.

### BACKGROUND OF THE INVENTION

#### (a) Field of the invention

The present invention relates to a liquid developer for use in developing an electrostatic latent image formed on an image-recording material by means of electrostatic charge. More particularly, the present invention relates to a liquid developer for use in developing said image in a single color and a set of liquid developers for use in developing said image in plural colors (or natural colors).

#### (b) Description of the prior art

A well-known method in the prior art is the so-called wet-process developing method which comprises the steps of (1) forming a latent image by electrostatic charge on an image-recording material such as a highly insulating plastic film or an electrophotographic copying material prepared by binding photoconductive powder onto the surface of a supporting sheet such as paper, a film, a metal sheet, etc. by means of a highly insulating resin, and then (2) dipping said image-recording material carrying the thus formed latent image in a developer prepared by dispersing electrostatically charged pigment particles in a liquid having a high electrical resistivity, thereby developing said latent image. As the electrostatically charged pigment particles, viz., the toner, one prepared by kneading carbon black with a natural rosin, an asphalt or a synthetic alkyd resin added thereto, thereby coating the former with the latter, is popular, while as the liquid having a high electrical resistivity, viz., the carrier liquid, a paraffinic hydrocarbon having an electrical resistivity more than  $10^9 \Omega \text{ cm.}$  and a dielectric constant less than 3 has hitherto been recommended. However, a liquid developer prepared by combining a toner and a carrier liquid as described above has been accompanied by such drawbacks that, in case of prolonged preservation or repeated use thereof, the coating agent is disengaged and separated from the pigment particles constituting the toner to effuse into the carrier liquid and, as a result, the toner fails to show a distinct electrification and dispersibility and finally presents a precipitation phenomenon, thereby hampering the completion of satisfactory developing.

Meanwhile, according to the currently popular copying

2

process employing liquid developers for plural-color (natural-color) electrophotography, a method has been adopted in which reproduction of the images and colors of an original is performed by repeating, say, three to four times or more often, an operation comprising the steps that, after impression of an electric charge on a copying material having a photoconductive layer by means of corona discharge, a colored original and a filter capable of selectively transmitting a desired color of said original image are superposed onto the thus processed copying material to effect exposure therethrough, whereupon the toner having said desired color is adsorbed onto the electrostatic latent image area formed as above. (The adsorption is usually effected by dipping said copying material in a liquid developer.) However, employment of such method in reproducing a plurality of colors onto the photoconductive layer of one and the same copying material has been accompanied by such a drawback that the toner (color) first adsorbed or adhered onto said photoconductive layer will effuse or be separated from the first developed image into the second developer containing the toner to be adsorbed next. Also, it has been accompanied by a drawback that said effusion or separation of toner would give rise to undesirable phenomena such as pollution of the second or succeeding developers, impairment of the color balance, etc. Consequently, when a colored image was formed on a copying material or an image-recording material by means of a set of developers for plural-color electrophotography consisting of a plurality of carrier liquids containing respectively toners of different colors, the color concentration of the first developed color-image area would become lower than that of the last developed image-area, and not only there would occur such pollution of the developers as set forth above, but also the definition of the copied image would not be satisfactory.

Such drawbacks of the prior art are attributable to the toner contained in the developer: that is, they are attributable to the fact that the substance employed for the purpose of providing the pigments of such colors as red, blue, yellow, black, etc. with polarity-controlling property, dispersibility and fixability was a rosin, an asphalt, an alkyd resin, or a vegetable oil. To be precise, when a pigment is coated with any of these substances and is dispersed in a carrier liquid, the greater part of such coating agent applied to the pigment effuses and the quantity thereof adhered to the surface of the pigment is reduced so as to become very small, thereby resulting in a diminished fixability of the toner to the image-recording material and finally causing the toner, which was previously adhered onto the surface of said image-recording material as described above, to effuse or separate therefrom to become present into the succeeding carrier liquid. Moreover, inasmuch as the foregoing developer has such a property that, when it is used repeatedly or stored for a long time, the coating agent employed therein gradually comes off the pigment, it would occasionally present such phenomena that the polarity of the toner would become indistinct or the toner would aggregate and to precipitate thereby making it impossible to reproduce the desired color.

In this context, the inventors have recently developed a toner prepared by directly graft-bonding the pigment and the coating agent so as to prevent the latter from coming off the former. But, in the case of a toner thus prepared, the substance applicable as the pigment is limited to a black material such as carbon black, Aniline Black and the like having a benzenoid ring, and, accordingly, though it has proved suitable as a monochromatic toner for providing black color, it has been still impossible to prepare toners of plural colors or a toner having various colors for use in developing a plural-color image. Moreover, since the quantity of the coating agent to be

graft-bonded to the pigment was strictly dependent on the conditions of the surface of pigment it was quite difficult to bond an ample coating agent in order to improve the fixability of the toner.

Further, said toner has also been defective in that the kind of said monomer or monomers to constitute the coating is extremely limited as it is required for the monomer or monomers to be bonded to said benzenoid ring and to act to provide the toner with afore-said properties (to wit, polarity-controlling property and dispersibility).

## SUMMARY OF THE INVENTION

The primary object of the present invention is to provide a liquid developer for use in electrostatic recording, which comprises a carrier liquid and a toner dispersed therein, said toner having an improved composition so as to be capable of employing a plurality of pigments as well as a polarity-controlling resin. The present invention has successfully overcome the defects of conventional toners by coating pigment particles with a coating agent which does not separate from said particles or deteriorate in its coating efficiency within said carrier liquid and graft-bonding a resin having a polarity-controlling effect and dispersing effect onto said coating agent. In other words, by composing a toner as above, not only does it become possible to employ a great variety of pigments as well as polarity-controlling resins for the toner, but also the developer containing the thus composed toner does not deteriorate in its developing efficiency even in case of repeated use and prolonged storage.

The second object of the present invention is to provide liquid developers for plural-color electrophotography comprising carrier liquid and toners of plural colors having a very strong fixability and separately dispersed in said carrier liquid for each color.

The developer according to the present invention is applicable not only to an electrostatic recording material having a photoconductive layer capable of forming a latent image thereon by impressing an electric charge and exposure as set forth above, but also to such an electrostatic recording material which is capable of directly forming thereon an electrostatic latent image corresponding to an original image by impressing an electric charge.

The toner according to the present invention consists of colored particles and a coating agent applied onto the surfaces of said particles together with a polymer grafted to said coating agent. Thus each toner particle is provided with a double-layer coating around said colored particle. But, inasmuch as said polymer is graft-bonded to the coating agent, it is possible to regard said double layer as a unitary layer.

As the colored particles to be employed in the present invention, either inorganic substances or organic substances are suitable. All of such colored substances called pigments and such colored substances called dyes are applicable. For example, as the black color particles, carbon black Color Index (C.I.) 77266, Aniline Black C.I. No. 50440 (a manufacture of Imperial Chemical Industries Ltd., England, hereinafter referred to as I Co.), Cyanine Black BX (a manufacture of Sumitomo Kagaku K.K.), Mogul A C.I. No. 77266, Elf Blacks C.I. No. 77266 and Elftex C.I. 77266 (manufactures of Godfrey L. Cabot, Inc., USA, as hereinafter referred to as C Co.), Spilon Black (a manufacture of Hodogaya Chemical Industries Ltd., hereinafter referred to as H Co.), Monolite Fast Black BX C.I. No. 50440 (a manufacture of I Co.), Spirit Black C.I. No. 50415 (a manufacture of Orient Chemical Industries Ltd., hereinafter referred to as O Co.), etc. are applicable. As the red-color particles, Spilon Red C.I. Solvent Red 8 (a manufacture of H Co.), Spilon Orange C.I. Solvent Orange 5 (a manufacture of H Co.), Benzine Orange C.I. No. 21110 (a manufacture of Sanyo Color Works Ltd., hereinafter referred to as S Co.), Brilliant Carmine 6B C.I. No. 15850 (a manufacture of S Co.), Scarlet KR C.I. No. 15865 (a manufacture of S Co.),

Co.), Fast Red C.I. No. 15865 (a manufacture of S Co.), Fast Rose 836 C.I. No. 45160 (a manufacture of Dainichi Seika K.K., hereinafter referred to as D Co.), Monolite Fast Red B (a manufacture of I Co.), etc. are applicable.

- Fast Red B (a manufacture of I Co.), etc. are applicable.

5 As for the yellow-color particles, Spilon Yellow C.I. Solvent Yellow 19 (a manufacture of H Co.), Benzine Yellow G NN C.I. No. 21100 (a manufacture of S Co.), Benzine Yellow 471 C.I. No. 21095 (a manufacture of D Co.), Monolite Fast Yellow IOG (a manufacture of I Co.), etc. are applicable. As for the blue-color particles, Victoria Blue C.I. Basic Blue 7 (a manufacture of H Co.), Methylene Blue C.I. Basic Blue 9 (a manufacture of H Co.), Oil Blue C.I. No. 61555 (a manufacture of O Co.), Alkali Blue C.I. No. 42750 (a manufacture of O Co.),

10 15 Sky Blue (a manufacture of S Co.), Cyanine Blue FG (a manufacture of S Co.), Cyanine Blue NSG C.I. No. 74250 (a manufacture of D Co.), Lignol Blue NCB (a manufacture of Toyo Ink Industries Ltd.), Monastral Fast Blue G (a manufacture of I Co.), Vali Fast Blue C.I. No. 74350 (a manufacture of O Co.), etc. are applicable. As for the green-color particles, Phthalocyanine Green LL (a manufacture of S Co.), Seika Light Green C.I. No. 42040 (a manufacture of D Co.), Phthalocyanine Green F7G C.I. No. 74260 (a manufacture of D Co.),

20 25 Chromofine Green G C.I. 74260 (a manufacture of D Co.), Phthalocyanine Green LX C.I. No. 42040 (a manufacture of S Co.), etc. are applicable. As for pigments of other colors than the foregoing, Spilon Violet C.I. Solvent Violet 2 (a manufacture of H Co.) is applicable

30 for a purple toner.

According to the present invention, these colored particles are coated with one kind or more than two kinds of coating agents for each color, said coating agent being selected from the group consisting of synthetic rubbers 35 such as acrylic rubber copolymer of styrene-butadiene, Pliolite VTL or VTAL rubbers (vinyl-toluene/butadiene rubbers), butylene rubber and styrene rubber, varieties of natural rubbers such as natural rubber-1135X (Malaya), Lacentex (Malaya), Minotex (Cambodia), Dunlop 40 (Malaya) and RCMA (Indonesia), polycondensates of said synthetic and natural rubbers, and polymers comprising at least one member of the group consisting of monomers to be expressed by the following general Formula 1.

The properties of the above natural rubbers are described in the Oct. 20, 1962 issue of "Kobunshi" (High Molecules) published by Kobunshi Gakkai (Society of High Molecules).

### General Formula 1



wherein, Y represents a radical selected from the group consisting of  $-\text{COOH}$ ,  $-\text{H}$  and  $-\text{Cl}$ ; and X represents a radical selected from the group consisting of



[wherein, L represents a radical selected from the group consisting of  $-\text{CH}_3$ ,  $-\text{NO}_2$ ,  $-\text{NH}_2$ ,  $-\text{N}(\text{CH}_3)_2$ ,  $-\text{COOH}$ ,  $-\text{COOCH}_3$ ,  $-\text{OH}$ ,  $-\text{OCH}_3$ ,  $-\text{Cl}$  and  $-\text{Br}$ ],



(wherein L is identical with said L),



(wherein, L is identical with said L, and n=1-4) and



(wherein, L is identical with said L, and n=1-4).

Any of these coating agents is insoluble in the carrier liquid for the developer as referred to later and, not only that, has such a property that it is easily graft-bonded to the below-mentioned monomers. Subsequent to being coated with such coating agent, the colored finely-divided particles are next graft-bonded respectively with such a monomer capable of forming a copolymer having an affinity with the carrier liquid and a solubility therein. As the monomer to be graft-bonded to said particles, it is selected from the group consisting of polymeric vinyl compounds and at least one member selected from the group consisting of such vinyl compounds as expressed by the following general Formula 2.

General Formula 2



wherein, R represents a radical selected from the group consisting of  $-\text{H}$  and  $-\text{CH}_3$ ; and R' represents a radical selected from the group consisting of alkyl radicals having 5 to 20 carbon atoms, cyclohexyl radical,  $-\text{OR}''$  (wherein R'' is identical with said radical R') and  $-\text{COOR}'''$  (wherein R''' represents a radical selected from the group consisting of alkyl radicals having 5 to 20 carbon atoms and cyclohexyl radical).

To give concrete examples of the compound expressed by said general Formula 2, there are enumerated such substances as vinyl stearate, vinyl laurate, vinyl oleate, tridecyl methacrylate, vinyl cyclohexylate, cyclohexyl acrylate, hexyl acrylate, heptacyl acrylate, dodecyl acrylate, octyl acrylate, stearyl acrylate, tridecyl acrylate, hexadecyl acrylate, n-amyl methacrylate, 2-ethylhexyl methacrylate, dodecyl methacrylate, heptadecyl methacrylate, hexyl methacrylate, stearyl methacrylate, lauryl vinyl ether, n-octyl vinyl ether, tridecyl vinyl ether, etc.

As the carrier liquid for the developer according to the present invention, any of the liquids containing liquid hydrocarbon of normal paraffin family, isoparaffin family, olefin family and naphtha family or said liquids combined with aromatic hydrocarbon, which are known as carrier liquids, for developers to be used in conventional wet-process developing method, are applicable. Said liquid hydrocarbon has an electrical resistivity not less than  $10^9 \Omega \text{ cm}$ . and a dielectric constant not greater than 3. To give examples of the hydrocarbon having such properties, there are such manufactures of ESSO Standard Oil Company as put on the market under tradenames of "Naphtha No. 6," "Solvesso 100," "Isopar-H," "Isopar-G" and "Isopar-L," and, besides, a manufacture of Mobil Oil Company sold under the trade-name "Pgasol AS-100." These manufacturers can be employed either individually or in mixtures of plural kinds thereof.

The developer according to the present invention is prepared by the below-mentioned treatment of the above-

described materials. That is, said colored particles and coating agent are first mixed with a solvent—preferably a solvent capable of dissolving said coating agent, such as toluene, benzene, or n-hexane—and subjected to kneading, and the kneaded mixture is then either subjected to spray-drying with a spray-dryer or dried and thereafter pulverized into finely-divided particles having a grain-size of  $1-5\mu$ . In this case, to make the mixing rate of said colored particles and coating agent to be 100 parts by

5 weight of the former against 100-500 parts by weight of the latter will serve for bonding of the monomer in comparatively large quantities on the occasion of the subsequent formation of graft-copolymers. Next, the particles thus coated with the coating agent are mixed with the 10 monomer to be graft-copolymerized, either in the presence of an appropriate solvent or no solvent, together with a reaction-initiator having a strong hydrogen-absorbability, such as benzoyl peroxide or lauryl peroxide, at a 15 temperature of  $100^\circ \text{ C}$ . or thereabout, whereby there 20 is prepared a toner consisting of said coated particle which surface is provided with a graft-polymer layer as chemically bonded thereon very firmly. Further, in case where the 25 reaction products brought about by the graft-polymerization reaction is hardened, they are pulverized into fine particles having a grain size of about  $1-5\mu$ . The mixing 30 rate of said coated particles and monomers for causing said graft-copolymerization is not particularly limited, but to make said mixing rate to be 100 parts by weight of the former against 50-500 parts by weight of the latter will 35 serve for effecting satisfactory provision of polarity-controlling property as well as dispersibility for the toner. And, the graft-polymerization reaction products are mixed in a carrier liquid having an intense affinity with the graft-copolymer layer and dispersed therein by 40 means of a ball-mill and the like, whereby a concentrated liquid developer is prepared.

By diluting the thus prepared concentrated liquid developer with at least one of those carrier liquids as 45 described above, there is obtained a liquid developer for use in developing an electrostatic latent image. Further, by diluting a concentrated liquid developer containing such toners prepared for each color as described above with respective carrier liquid, there is obtained liquid developer for plural-color development in one set of 50 developers for four colors of black, yellow, blue and red. 55 And, in case where the toner for a single color is employed, the liquid developer can be made into a liquid developer for monochromatic development.

In case of the thus prepared developer according to the 55 present invention, the toner contained therein is coated with an increased amount of graft-polymer as compared with conventional toners, and this coating does not come off or effuse into the carrier liquid, so that the fixability thereof is great. Therefore, in case of reproducing a 60 plural-color image, even after repeated dipping in the developer, the toner once fixed onto an electrostatic recording material does not come off into another developer. Thus, there is no fear of the color balance being impaired or the non-image area being stained, so that 65 a faithful reproduction of the plural-color image of the original can be expected. Moreover, inasmuch as the graft-polymer portion of the toner is chemically bonded directly onto the coating having an insolubility against the carrier liquid, its bonding with the colored particles is firm and its affinity with the carrier liquid is great, and as a result, even after a prolonged storage and repeated use thereof, the toner can display a satisfactory dispersibility and does not show any deterioration of the polarity-controlling effect thereof. And, a monochromatic or polychromatic copied image formed by employing the developer according to the present invention, when employed for transfer onto another supporting material by means of a strong solvent, is capable of being easily transferred, and the definition of thus transferred image is also satisfactory.

## DESCRIPTION OF THE PREFERRED EMBODIMENTS

## Example 1

|                                    |     |     |
|------------------------------------|-----|-----|
| A mixture, prepared by kneading:   | Kg. | 5   |
| Carbon black                       |     | 1   |
| Styrene-butadiene copolymer rubber |     | 2.5 |
| Toluene                            |     | 6.0 |

was subjected to spray-drying with a spray-dryer, whereby 10 copolymer-coated particles having a grain-size of about 1-5 $\mu$  were prepared. To 500 g. of said particles were added 300 g. of hexyl methacrylate and 10 g. of benzoyl peroxide, and these substances were mixed with one another at a temperature of 115-120° C. for 24 hours, 15

sequently, 100 g. of thus obtained graft-reaction products was added to 500 g. of Naphtha No. 6 and mixed with each other for 20 hours in a ball-mill. Thereafter, 20 g. of the resultant mixture was dispersed in 1000 ml. of Naphtha No. 6, whereby there was obtained a liquid developer containing the toner charged positively.

The efficiency of thus obtained liquid developer has proved equivalent to that of the developer prepared in Example 1.

## Example 3

According to those manufacturing processes for developer in Examples 1 and 2 and by applying those combinations of material as shown in the following Table I, a variety of liquid developers were prepared.

TABLE I

| Developer No. | Colored particles | Coating agent                                                 | Monomer for graft-polymerization | Carrier liquid                 | Polarity of toner |
|---------------|-------------------|---------------------------------------------------------------|----------------------------------|--------------------------------|-------------------|
| 1             | Victoria blue     | Vinyl toluene-methyl methacrylate copolymer(mol ratio 8:2)    | Heptacylmethacrylate             | Isopar G                       | Positive          |
| 2             | Phthalocyanine    | Acrylonitrile-parachlorostyrene(mol ratio 2:8)                | Cyclohexyl acrylate              | Naphtha No. 6                  | Do.               |
| 3             | Spirit black      | Glycidyl methacrylate para-amino styrene (mol ratio 3:7)      | Vinyl laurate                    | Naphtha No. 6/Isopar H=6/4     | Do.               |
| 4             | Spilon yellow     | Hydroxyl methacrylate 2,5-hydroxy styrene (mol ratio 4:6)     | Tridecyl vinyl ether             | Isopar H                       | Do.               |
| 5             | Benzine yellow    | Dimethylaminoethyl methacrylate-vinyl benzoate(mol ratio 5:5) | Vinyl cyclooctylate              | Naphtha No. 6/toluene=8/2      | Do.               |
| 6             | Cyanine blue      | Acrylamide-2,4-dichlorostyrene(mol ratio 4:6)                 | Stearyl methacrylate             | Solvesso 100/Naphtha No. 6=6/4 | Do.               |

thereby effecting graft-polymerization reaction. Subsequently, the graft-reaction product was pulverized into particles having a grain size of about 1 $\mu$ , whereby a toner was prepared. Then, to 500 g. of a carrier liquid prepared by mixing 8 parts by weight of Naphtha No. 6 with 2 parts by weight of Solvesso 100, 100 g. of said toner was added, and they were mixed with each other in a ball-mill for 24 hours. Thereafter, 10 g. of thus prepared mixture was dispersed in 1000 ml. of Naphtha No. 6, whereby 30 there was obtained a liquid developer containing the toner charged positively.

A commercialized electrostatic recording paper prepared by forming a photoconductive layer on a supporting paper by means of binding zinc oxide powder thereon with a resinous binder was first impressed with negative charge by corona discharge, and thereafter an original having a desired image was superposed onto thus impressed recording paper to effect exposure. When said recording paper was dipped in the abovementioned developer subsequent to exposure, there was formed a clear-cut positive copied image reproducing faithfully said original image. Further, even in case where about 5000 sheets of the recording paper were developed through the same process as above by employing one and the same developer over 12-month period, there was no trace of deterioration of the electrification property of the toner nor any aggregation thereof, and it was possible to obtain copied images having the same definition as rendered by the developer in the initial stage subsequent to manufacturing thereof. The image-area thus developed by the developer according to the present invention is possessed of a splendid fixability, so that, even when rubbed with fingers, the toner will not come off, nor will the non-image area become stained, either.

## Example 2

|                                                                                    |      |
|------------------------------------------------------------------------------------|------|
| A mixture, prepared by kneading:                                                   | Kg.  |
| Brilliant Carmine 6B                                                               | 2    |
| Styrene-butyl methacrylate copolymer (mol ratio of styrene/butyl methacrylate=1/3) | 4.5  |
| Benzene                                                                            | 10.0 |

was subjected to spray-drying with a spray-dryer, whereby copolymer-coated particles having a grain-size of about 1-5 $\mu$  were prepared. To 500 g. of said particles were added 400 g. of lauryl methacrylate and 12 g. of lauroyl peroxide, and these substances were mixed with one another at a temperature of 105-115° C. for 30 hours, 70 thereby effecting graft-polymerization reaction. Subse-

sequently, 100 g. of thus obtained graft-reaction products was added to 500 g. of Naphtha No. 6 and mixed with each other for 20 hours in a ball-mill. Thereafter, 20 g. of the resultant mixture was dispersed in 1000 ml. of Naphtha No. 6, whereby there was obtained a liquid developer containing the toner charged positively.

## Example 4

The following examples pertain to the explanation of a set of liquid developers for plural-color development wherein each toner of black, yellow, blue and red is dispersed in separate carrier liquid for each color.

## (a) Preparation of a developer containing black-color toner

|                                  |     |
|----------------------------------|-----|
| A mixture, prepared by kneading: | Kg. |
| Carbon black                     | 1   |
| Styrene-butadiene copolymer      | 3   |
| Toluene                          | 6   |

was subjected to spray-drying with a spray-dryer, whereby copolymer-coated particles having a grain-size of about 1-5 $\mu$  were prepared. To 500 g. of said particles were added 350 g. of n-amyl methacrylate, 500 g. of n-hexane and 6.5 g. of benzoyl peroxide, and these substances were mixed with one another at a temperature of 110-115° C. for 12 hours, thereby effecting graft-polymerization reaction. Subsequently, 100 g. of thus obtained graft-reaction products were added to 500 g. of a mixed carrier liquid prepared by mixing 8 parts by weight of Naphtha No. 6 with 2 parts by weight of Solvesso 100, and they were mixed in a ball-mill for 24 hours, whereby a concentrated toner solution was prepared. Then, 10 g. of said toner solution were dispersed in 1000 ml. of Naphtha No. 6, whereby there was obtained a liquid developer containing black-color toner charged positively.

## (b) Preparation of a developer containing yellow-color toner

|                                                                                                 |     |
|-------------------------------------------------------------------------------------------------|-----|
| A mixture, prepared by kneading:                                                                | Kg. |
| Spilon Yellow                                                                                   | 1.0 |
| Methacrylic acid - hydroxyl ethyl methacrylate-butyl methacrylate (mol ratio=1:0.2:5) copolymer | 2.1 |
| Solvesso 100                                                                                    | 4.0 |

was treated in the same way as in case of preparing the foregoing black-color toner, whereby copolymer-coated particles having a grain-size of about 1-5 $\mu$  were prepared. To 100 g. of said coated-particles were added 80 g. of 2-ethyl hexylmethacrylate and 0.5 g. of benzoyl peroxide, and these substances were mixed with one another at a temperature of 115-120° C. for 8 hours, thereby effecting graft-polymerization reaction. Subsequently, 50 g. of

thus obtained graft-reaction products were added to 400 g. of Naphtha No. 6 and mixed with each other in a ball-mill for 16 hours, whereby a concentrated yellow-color toner solution was prepared. Then, 30 g. of said toner solution were dispersed in 1000 ml. of Naphtha No. 6, whereby there was obtained a liquid developer containing yellow-color toner charged positively.

(c) Preparation of a developer containing blue-color toner

A mixture, prepared by kneading:

|                                                      | Kg. |
|------------------------------------------------------|-----|
| Cyanine Blue NSG                                     | 0.5 |
| Styrene-butyl methacrylate (mol ratio=4:6) copolymer | 1.2 |
| Toluene                                              | 1.5 |

was treated in the same way as in case of preparing the foregoing black-color toner, whereby copolymer-coated particles having a grain-size of about  $1-5\mu$  were prepared. To 200 g. of said coated particles were added 30 g. of methacrylic acid, 120 g. of lauryl methacrylate and 2.5 g. of lauroyl peroxide, and these substances were mixed with one another at a temperature of 115-125° C. for 16 hours, thereby effecting graft-polymerization reaction. Subsequently, 100 g. of thus obtained graft-reaction products and 500 g. of Naphtha No. 6 were mixed with each other in a ball-mill for 18 hours, whereby a concentrated blue-color toner solution was prepared. Thereafter, 15 g. of said toner solution were dispersed in 1000 ml. of Naphtha No. 6, whereby there was obtained a liquid developer containing blue-color toner charged positively.

(d) Preparation of a developer containing red-color toner

A mixture, prepared by kneading:

|                                                                  | Kg. |
|------------------------------------------------------------------|-----|
| Brilliant Carmine 6B                                             | 1.5 |
| Glycidyl methacrylate - vinyl toluene (mol ratio =2:8) copolymer | 4   |
| Toluene                                                          | 1.0 |

was subjected to spray-drying as set forth in the foregoing, whereby copolymer-coated particles having a grain-size of about  $1-5\mu$  were prepared. To 200 g. of said coated particles were added 50 g. of cyclohexyl methacrylate, 100 g. of tridecyl methacrylate, 0.6 g. of lauroyl peroxide, 0.4 g. of benzoyl peroxide and 100 g. of Naphtha No. 6, and these substances were mixed with one another at a temperature of 115-120° C. for 48 hours, thereby effecting graft-polymerization reaction. Subsequently, 100 g. of thus obtained graft-reaction products were added to 500 g. of a mixed carrier liquid prepared by mixing 8 parts by weight of Naphtha No. 6 with 2 parts by weight of Isopar H, and they were mixed in a ball-mill for 16 hours, whereby a concentrated red-color toner solution

was prepared. Then, 15 g. of said toner solution were dispersed in 100 ml. of Naphtha No. 6, whereby there was obtained a liquid developer containing red-color toner charged positively.

- 5 By employing a set of liquid developers for plural-color electrophotography prepared as above and conventionally processing a commercialized electrophotographic copying paper (viz., a copying paper prepared by forming a photoconductive layer on a supporting paper by means of 10 binding zinc oxide powder thereon with a resinous binder), a plural-color image was reproduced. To be precise, the photoconductive layer of said copying paper was first impressed with negative electrostatic charge, and thereafter filters for green, red and blue colors were interposed between a plural-color original and said electrified 15 copying paper, whereby exposure was conducted. Thus exposed copying paper was then dipped in the afore-said developer containing the black-color toner, whereby the black image-area was first formed. Said copying paper 20 having thus formed black image-area was impressed with electrostatic charge, subjected to exposure through a red-color filter interposed between a plural-color original and said copying paper, and then dipped in the developer containing the yellow-color toner, whereby the yellow image-area was formed. Subsequently, by applying successively such processes that impression of electronic charge, exposure through a green-color filter, dipping in the developer containing red-color toner, another impression of electrostatic charge, exposure through a blue-color filter, and dipping in the developer containing blue-color toner in order, there was obtained a distinct plural-color copied-image reproducing said plural-color original faithfully. 25 The plural-color copied-image thus reproduced would not show any coming-off of the toner even when rubbed intensely with fingers, nor would the non-image area get stained, either.

Further, even in case where 3000 sheets of said copying paper were developed successively over 12-month period by employing a single set of such developers as prepared 40 in the present example, it was possible to reproduce plural-color images having such definition as by no means inferior to that rendered by the developers in the initial stage subsequent to manufacturing thereof.

Example 5

By applying those combinations of materials as shown in the following Table II and according to those methods of preparing developers in Example 4, 4 sets of liquid developers for plural-color electrophotography were prepared.

TABLE II

| De-<br>vel-<br>oper<br>No. | Materials for toner |                                                           |                                         |                                  | Polarity<br>of toner |
|----------------------------|---------------------|-----------------------------------------------------------|-----------------------------------------|----------------------------------|----------------------|
|                            | Colored particles   | Coating agent                                             | Monomer for graft-<br>polymerization    | Carrier liquid                   |                      |
| 1                          | Aniline black       | Orthochlorostyrene-acrylonitrile copolymer.               | Cycloheptacyl methacrylate              | Isopar H                         | Positive.            |
|                            | Spilon yellow       | Para-aminostyrene-methyl methacrylate-butyl methacrylate. | Lauryl vinyl ether                      | do                               | Do.                  |
|                            | Spilon red          | Para-nitrostyrene-2-chloroethyl acrylate.                 | n-Tetradecyl methacrylate               | do                               | Do.                  |
|                            | Victoria blue       | Para-hydroxyl styrene-propyl methacrylate.                | n-Hexyl vinyl ether                     | Naphtha No. 6                    | Do.                  |
| 2                          | Spirit black        | 2,4-dimethyl styrene-N,N-dimethyl acrylamide.             | 4-pentene                               | do                               | Do.                  |
|                            | Benzine yellow 471  | 2,4-dichlorostyrene-glycidyl methacrylate.                | Cyclopentacyl acrylate                  | do                               | Do.                  |
|                            | Spilon orange       | Para-dimethylamino-styrene-acrylic acid.                  | Stearyl vinyl ether                     | Isopar G                         | Do.                  |
|                            | Alkali blue         | Para-methoxystyrene-2-chloro-methyl acrylate, Dunlop.     | 1-octene                                | do                               | Do.                  |
| 3                          | Spilon black        | Para-carboxylstyrene-arylacrylate.                        | Vinyl olate                             | Naphtha No. 6/Solvesso 100 (8/2) | Do.                  |
|                            | Benzine yellow TG   | Para-phenylstyrene-isobutyl methacrylate.                 | 1-nonene                                | Naphtha No. 6/Solvesso 100 (9/1) | Do.                  |
|                            | Fast red            | Para-bromostyrene-hydroxyl ethyl methacrylate.            | Cyclopentacyl acrylate                  | Naphtha No. 6/Solvesso 100 (7/3) | Do.                  |
|                            | Cyanine blue        | Para-phenoxystyrene-vinyl butylate.                       | 2-ethyl-hexyl acrylate                  | Isopar H                         | Negative.            |
| 4                          | Carbon black XO-550 | 2,3-dinitrostyrene-vinyl phthalate                        | Octyl vinyl ether                       | Isopar G                         | Positive.            |
|                            | Benzine yellow GNN  | Orthonitrostyrene-acryl vinyl ether.                      | 3-hexene                                | Naphtha No. 6/Solvesso 100 (6/4) | Do.                  |
|                            | Scarlet KR          | Para-cyclohexyl styrene-vinyl acetate.                    | Octadecyl methacrylate                  | Naphtha No. 6                    | Do.                  |
|                            | Phthalocyanine blue | Glycidyl methacrylate-acrylic acid-styrene.               | Cyclohexyl vinyl ether (vinyl stearate) | do                               | Positive (negative). |

The efficiency of any of these 4 sets of developers has proved equal to that of those developers in Example 4.

What we claim is:

1. A method for manufacturing a liquid developer for use in electrophotography, which comprises the steps of:
  - (a) kneading particles of a colored substance selected from the group consisting of dyes and pigments, and
  - (b) at least one coating agent selected from the group consisting of (i) a synthetic rubber selected from the group consisting of acrylic rubber, copolymers of styrene-butadiene, vinyl toluene-butadiene rubber, butylene rubber and styrene rubber, (ii) natural rubber, (iii) poly-condensates of said synthetic rubber and natural rubber and (iv) polymers prepared by polymerizing at least one monomer of the

Formula 1



5

10

15

20

wherein, Y is selected from the group consisting of  $-\text{COOH}$ ,  $-\text{H}$  and  $-\text{Cl}$ ; and X is selected from the group consisting of  $-\text{C}_n\text{H}_{2n+1}$  ( $1 \leq n \leq 4$ ),  $-\text{OCOC}_n\text{H}_{2n+1}$  ( $1 \leq n \leq 4$ ),  $-\text{OC}_n\text{H}_{2n+1}$  ( $1 \leq n \leq 4$ ),  $-\text{CN}$ ,  $-\text{COOH}$ ,  $-\text{Cl}$ ,  $-\text{COCl}$ ,  $-\text{COOR}$  (wherein R is selected from the group consisting of  $-\text{C}_n\text{H}_{2n+1}$  ( $1 \leq n \leq 4$ ),



30

and



35

40

45

(wherein, L is selected from the group consisting of  $-\text{CH}_3$ ,  $-\text{NO}_2$ ,  $-\text{N}(\text{CH}_3)_2$ ,  $-\text{COOH}$ ,  $-\text{COOCH}_3$ ,  $-\text{OH}$ ,  $-\text{OCH}_3$ ,  $-\text{Cl}$  and  $-\text{Br}$ )



(wherein L has the same meaning as above),  $-\text{(CH}_2)_n$



- 12  
(wherein L has the same meaning as above and  $n=1-4$ ) and  $-\text{CH}_2)_n$



(wherein L has the same meaning as above and  $n=1-4$ ); pulverizing the resultant mixture into finely divided particles coated with said coating agent; mixing said finely divided first coated particles and a vinyl monomer of the



wherein, R is selected from the group consisting of  $-\text{H}$  and  $-\text{CH}_3$ ; and R' is selected from the group consisting of alkyl radicals having 5 to 20 carbon atoms, cyclohexyl,  $-\text{OR}''$  (wherein R'' has the same meaning as R') and  $-\text{COOR}'''$  (wherein R''' is selected from the group consisting of alkyl radicals having 5 to 20 carbon atoms); polymerizing said monomer in the mixture thus obtained in the presence of a reaction initiator having a strong hydrogen absorbability to form on said coated particles a second coating; pulverizing the resultant reaction product into fine particles having a grain size of about  $1-5\mu$ ; and then dispersing said fine particles into a carrier liquid consisting of a liquid hydrocarbon having an electrical resistivity not less than  $10^9\Omega$  cm. and a dielectric constant not greater than 3.

2. A method according to claim 1, wherein the mixing ratio of said colored substance and said coating agent is in the range of from 100 to 500 parts by weight of the latter per 100 parts by weight of the former.

3. A method according to claim 2, wherein the mixing ratio of said finely-divided particles coated with said coating agent and said monomer is in the range of from 50 to 500 parts by weight of the latter per 100 parts by weight of the former.

#### References Cited

##### UNITED STATES PATENTS

|           |         |               |       |          |
|-----------|---------|---------------|-------|----------|
| 3,503,881 | 3/1970  | Shinohara     | ----- | 252—62.1 |
| 3,133,893 | 5/1964  | Newman        | ----- | 252—41   |
| 3,471,439 | 10/1969 | Bixler et al. | ----- | 260—41   |
| 3,325,409 | 6/1967  | Whitbread     | ----- | 252—62.1 |
| 3,090,755 | 5/1963  | Erchak et al. | ----- | 252—62.1 |

GEORGE F. LESMES, Primary Examiner

J. P. BRAMMER, Assistant Examiner

U.S. Cl. X.R.

96—1.2; 106—308 M; 260—41 C, 41.5 R